

Aug. 5, 1958

J. N. DEMPSEY

2,846,339

METHOD OF FORMING AN ELECTRON EMITTING BODY

Filed Oct. 21, 1953



INVENTOR.

JOHN N. DEMPSEY

BY

*Orvin M. Hagan*  
ATTORNEY

1

2,846,339

METHOD OF FORMING AN ELECTRON  
EMITTING BODY

John N. Dempsey, Edina, Minn., assignor to Minneapolis-Honeywell Regulator Company, Minneapolis, Minn., a corporation of Delaware

Application October 21, 1953, Serial No. 387,515

4 Claims. (Cl. 117—223)

The present invention relates to an improved electron emissive cathode having superior electrical and mechanical properties, and to the method of producing the same. More specifically, this invention relates to an improved dispenser-type cathode which includes a porous matrix impregnated throughout with an oxide of an alkaline earth metal capable of activation to form a composite of the alkaline earth metal and the oxide thereof; the porous base metal matrix being sintered and formed to its final desired shape before the impregnation procedure.

The present invention is an improvement over the co-pending application of Edward F. Rexter, Serial No. 387,537, filed October 21, 1953, assigned to the same assignee as the present invention and entitled Electron Emitting Cathodes.

According to present day methods of producing electron emitting cathodes, the emitting material for example, barium-strontium oxide, is sprayed onto, brushed onto, or mechanically compressed directly into the cathode base metal matrix. This oxide coating may be applied directly to the cathode body as such, or, it may be applied in the form of a carbonate and subsequently converted to the oxide. Although these procedures have met with general approval, they leave room for considerable improvement, particularly since these cathodes are subject to rapid deterioration due to the tendency of the emissive coating to peel or flake away from the matrix after short periods of operation. This deficiency is even more pronounced when the unit is subjected to periods of rough handling or operation. Basically, there is insufficient adherence between the base metal matrix and the emissive coating in these present day devices, and the coating is thus subject to deterioration, particularly in instances of mechanical vibration or shock. Of course, when this emissive coating breaks away from the cathode body, there is no additional emissive material available, and the cathode as well as the device with which it is being operated, for example, a vacuum tube is rendered useless.

The present invention provides an extremely rugged type of dispenser cathode in which the emissive coating tenaciously adheres or bonds itself to the matrix body without need for an adhesive or bonding agent, and it is able to endure severe vibration and shock without peeling away or flaking off. In accordance with the present invention, the emissive coating forms as a continuous layer or "continuum" within the porous matrix which also has a continuous structure or "continuum" of metal throughout its extent. In addition, a higher ratio of emission per unit area of cathode is achieved than is possible with conventional cathodes, thus, smaller cathodes may be utilized for a given rate of emission in accordance with the present invention. Further, a low interface resistance between the base metal matrix and the emissive coating is obtained when the elements are made in accordance with the present invention.

The present invention provides an extremely simple and efficient method of impregnation which may be accom-

2

plished with a single-step impregnation procedure, thereby eliminating possible sources of contamination.

Therefore, it is an object of the present invention to produce an improved electron emitting cathode having an electron emitting substance which is tenaciously bonded to the surface of the base metal matrix, thus producing a more rugged type of cathode structure.

It is a further object of the present invention to produce an electron emitting cathode which is able to endure mechanical shock and vibration without losing the emissive coating through flaking or peeling.

It is still a further object of the present invention to provide an electron emitting cathode which has a substantially continuous supply of emitting material available for the electron emitting body.

An additional object of the present invention is to provide a dispenser-type electron emitting cathode which has a low interface resistance between the matrix body and the electron emitting substance.

It is still a further object of the present invention to provide an improved method of producing electron emitting cathodes which employ a single-step impregnation procedure, and produce a very tightly adhering alkaline earth metal oxide coating on a base metal matrix.

Reference is made to the accompanying drawing which shows in block diagram form a flow sheet of a suggested process in accordance with the present invention.

According to present invention, a porous base metal matrix is prepared in accordance with conventional metallurgical procedures. For example, powdered nickel or any other suitable oxide cathode base metal is thoroughly mixed with a volatile binder, and a slurry made therefrom. The slurry, preferably being of pasty consistency, is then placed in a die and pressed with sufficient pressure to compress the slurry into the desired form. I prefer to use relatively low compressing pressures in order that the resulting matrix body may be highly porous. The pressed bodies are then sintered under a neutral or reducing atmosphere, for example, hydrogen, the binder preferably being volatilized at the sintering temperature so as to leave a porous base metal matrix. This matrix is then cleaned to remove impurities therefrom and is then ready for impregnation. When nickel is employed as the base metal, a matrix produced therefrom having a "porosity" of 20 to 50% is satisfactory. "Porosity" is defined as:

$$P = \left(1 - \frac{D_1}{D_2}\right) 100$$

wherein:

$P$  = porosity in percent

$D_1$  = weight of base metal matrix per volume of matrix

$D_2$  = density of base metal

As a general rule, as the powder size decreases the number of pores increases, which is desirable. For example, in a nickel base metal powder having a size ranging from 37 to 44 microns a porosity of 27.4% has been found satisfactory, whereas a powder size having a range of under 37 microns, pressing to a porosity of 29.2% was very satisfactory. It should be noted at this point, however, that a relatively high degree of porosity is desired in the base metal matrix since this creates a body wherein a substantial amount of the inner-pores are accessible from the outer surface of the body. This is based upon the impregnation step which follows.

In general, impregnation is carried out in a single step or operation, this step comprising introduction of a solution of a soluble thermally decomposable alkaline earth salt which is capable of thermal decomposition to the oxide thereof, for example, the soluble alkaline earth metal salts of organic acids which are thermally decom-

posable to the oxide thereof. After impregnation, the base metal matrix is subjected to a temperature sufficient to decompose the alkaline earth metal salt to the oxide thereof. The volatile by-products of the decomposition are preferably removed as formed. Generally, the salts decompose to the carbonate which is then further decomposed to the oxide by heating to a sufficiently high temperature. After conversion to the oxide, the cathode is ready for activation. Activation may be accomplished by heating the oxide impregnated cathode body in the presence of a reducing agent to produce a quantity of free alkaline earth metal in the alkaline earth oxide. For example, activation is accomplished by heating the impregnated cathode body to a temperature of from 1000° C. to 1200° C. for a period of time sufficiently long to activate the body, but not for such a long period as will evaporate an appreciable amount of the activating material. For example, I have found that an activating period of from 2 to 3 minutes under these conditions is satisfactory. Where barium and strontium oxide is present in the cathode body, the activation reduces a portion of these oxides to the free metal, the barium being reduced in greater proportion than the strontium. Thus, there is created a continuous body or continuum of free alkaline earth metal and the oxide thereof. It is preferable to hold the element out of contact with gases such as air in order to prevent the recombination of the oxide with carbon-dioxide or water, thus forming undesirable impurities in the cathode structure.

When a nickel base metal cathode matrix is employed, small amounts of aluminum may be present as a residual or added element. This aluminum acts as a reducing agent in the matrix and has been found satisfactory.

In accordance with the preferred modification of the present invention, a porous base metal matrix, prepared as above indicated is impregnated with a solution of barium and strontium acetates. A saturated solution of 50/50 mol ratio is preferred. This impregnation may be carried out by simply immersing the base metal matrix in the solution until the required amount of salt is contained in the matrix, or by placing the solution, for example by eye-dropper, onto the surface of the raw body. I prefer to utilize a sufficient amount of thermally decomposable salt in this step to provide for between 1 and 10% by weight of alkaline earth metal oxide in the porous base metal matrix. Following the impregnation, the matrix body is dried and then subjected to a heat treatment wherein the acetate salts are decomposed to the carbonates according to the following equations:



Heating to a temperature of 1000° C. is generally sufficient for the first reaction to go to completion. The symmetrical ketone is preferably removed from the reaction chamber as quickly as possible, that is, on formation. After the acetates have been completely converted to the carbonates by purely thermal means, the temperature is increased to 1150° C. at which temperature the carbonates are decomposed into the respective oxides, the carbon dioxide by-product being removed as it is formed.

This impregnation may also be accomplished by a modified procedure. In this modified procedure, barium and strontium formate are impregnated into the porous matrix as in the case of the acetate salts. They are then decomposed according to the equations,



Another modification of the procedure may be carried

out by utilizing the acetate-formate salt, according to the following reaction.



Similar equations may be written for the corresponding strontium salts. This modified procedure has some advantage over the acetate method in that the acetaldehyde boils at a lower temperature than does acetone. It is to be noted, however, that closer control is necessary in this modification since the reaction is somewhat violent unless some care is taken to volatilize off the acetaldehyde relatively slowly.

Various other modifications are possible wherein soluble alkaline earth metal salts of higher organic acids are utilized, for example, the propionate and butyrate. In this case, if a single salt is used, the by-product formed is the symmetrical ketone, a mixture of these higher salts yields an unsymmetrical ketone; and in case any of these salts are utilized in conjunction with the formate, the by-product formed is the corresponding aldehyde. After decomposition of the carbonate to the oxide in each of these cases, the cathode body is activated as previously described.

If desired, the cathode matrix may be first mounted in its assembly, regardless of its complexity, and thereafter impregnated in accordance with the materials and methods set forth above with the additional utilization of an eye-dropper to dispatch the solutions onto the base metal matrix where desired. Such a procedure is readily adaptable to production methods.

Many details of process and procedure may be varied without departing from the principles of this invention. It is therefore not my purpose to limit the scope of this invention other than necessitated by the scope of the appended claims.

I claim as my invention:

1. The method of forming an electron emitting body which includes the steps of impregnating a porous metal sponge matrix with an aqueous solution of an alkaline earth metal formate and an alkaline earth metal acetate, said formate and said acetate being employed in substantially equi-molar proportions, thermally decomposing said salts to the oxide form in-situ and then activating said oxide impregnated matrix to create electron emitting characteristics.

2. The method of producing an electron emitting cathode which includes the steps of impregnating a porous base metal pellet with an aqueous solution of barium-strontium acetate and barium-strontium formate said acetate and formate being in substantially equi-molar proportions, thermally decomposing said salts to the oxide form, and then activating said oxide impregnated matrix to create electron emitting characteristics.

3. The method as defined in claim 2 being further characterized in that said porous metal pellet consists essentially of nickel.

4. The method of producing an electron emitting cathode which includes the steps of impregnating a nickel pellet with an aqueous solution of barium-strontium acetate and barium-strontium formate, said acetate and formate being in substantially equi-molar portions, thermally decomposing said salts to the oxide, and then activating said oxide impregnating matrix by heating to a tempera-

ture of 1000° C. to 1200° C. in the presence of a reducing agent.

References Cited in the file of this patent

UNITED STATES PATENTS

1,532,533 Harris Apr. 7, 1925  
1,894,059 Ruffley Jan. 10, 1933

1,939,075  
1,981,245  
2,085,605  
2,389,060  
2,456,649  
2,525,263  
2,769,708

McCulloch Dec. 12, 1933  
Pearcy Nov. 20, 1934  
Ramsey et al. June 29, 1937  
Kurtz Nov. 13, 1945  
Rouse Dec. 21, 1948  
Macksoud Oct. 10, 1950  
Coppola et al. Nov. 6, 1956